

S. O. COWPER-COLES.  
SCALING, ANNEALING, AND COATING METALS.  
APPLICATION FILED OCT. 29, 1909.

979,931.

Patented Dec. 27, 1910.

2 SHEETS—SHEET 1.



Fig. 1

Witnesses.

J. H. Moore

R. E. Barry

Inventor.

S. O. Cowper-Coles

Redeemer of the world  
at the age of 82

S. O. COWPER-COLES.  
SCALING, ANNEALING, AND COATING METALS.  
APPLICATION FILED OCT. 29, 1909.

979,931.

Patented Dec. 27, 1910.

2 SHEETS—SHEET 2.



Witnesses.

J. A. Groome  
R. E. Barry.

Inventor.

Seward O. Cowper-Coles  
by  
Wm. W. Cowper-Coles.

# UNITED STATES PATENT OFFICE.

SHERARD OSBORN COWPER-COLES, OF WESTMINSTER, LONDON, ENGLAND, ASSIGNOR  
OF ONE-HALF TO METALLOIDS LIMITED, OF TIPTON, ENGLAND, A COMPANY.

## SCALING, ANNEALING, AND COATING METALS.

979,931.

Specification of Letters Patent. Patented Dec. 27, 1910.

Application filed October 29, 1909. Serial No. 525,309.

To all whom it may concern:

Be it known that I, SHERARD OSBORN COWPER-COLES, a subject of the King of Great Britain, residing at Grosvenor Mansions, 82 Victoria street, Westminster, London, England, have invented new and useful Improvements in Scaling, Annealing, and Coating Metals, of which the following is a specification.

10 This invention relates to an improvement in removing scale and oxid from metallic surfaces and annealing the cleansed metal which may also, when desired, be coated with zinc, tin or other metal.

15 My invention has for its object to overcome the disadvantage attaching to processes hitherto proposed and to this end I employ gases such as Mond-gas, producer-gas, Riché wood gas, water gas, or the vaporized lower 20 members of the paraffin and alcohol series, and I heat the metal surface to be cleaned to the annealing temperature and in some cases above the annealing temperature, in a large excess of such reducing gas, the 25 water vapor which is generated during the reduction of the metallic scale or oxid being prevented from condensing in any part of the apparatus by maintaining the ends of the apparatus, that is to say, those portions 30 through which the material to be scaled enters and leaves, at a temperature of 100° to 150° C. by which means the water vapor which is formed passes out of the apparatus with the excess of reducing gas. The scaled 35 and annealed metals may subsequently be coated with zinc, tin or the like in which case the scaling gases may be freed from sulfur compounds by being passed through a solution such as copper sulfate or caustic 40 potash and from unsaturated hydrocarbons by being passed through strong sulfuric acid; the combined processes being carried out in a suitable apparatus, for example, the apparatus mentioned in the former British 45 specification No. 28636 of 1907.

In carrying out my invention as applied for example to the cleaning, annealing and galvanizing of iron sheets or wire, I advantageously proceed as follows: The sheet 50 or wire to be treated is drawn into the heating chamber through a suitable opening, sealed or otherwise, the chamber being heated to the required temperature for annealing and in some cases above that temperature as hereinafter described; when using

the reducing gases not freed from sulfur compounds or unsaturated hydrocarbons it is necessary to heat the chamber to a higher temperature than that necessary when scaling with the gases freed from sulfur compounds and unsaturated hydrocarbons. Any scale or oxid which may be present on the sheet or wire is reduced to the metallic state during the passage through the chamber.

60 After its passage through the annealing chamber the sheet or wire is drawn into a cooling chamber where its temperature is lowered to a suitable point for running into the air for subsequent coating or directly into the bath of molten metal beneath the 65 surface of which the sheet or wire is drawn by any convenient means such as roller mechanism. On leaving the bath the cleaned annealed and coated metal is passed through 70 a second suitable opening sealed or otherwise 75 into the atmosphere.

It will be understood that the reducing gases referred to are passed through the scaling and annealing apparatus or the scaling, annealing and coating apparatus and 80 may in either case be finally employed for heating.

In order that my invention may be clearly understood, I have illustrated in the accompanying drawings, one form of apparatus by which my process may be carried out, similar letters of reference indicating 85 identical parts throughout, and in which:—

Figure 1 is a longitudinal section of apparatus for carrying out the process herein 90 described. Fig. 2 is a plan view thereof.

*a* indicates the wire to be treated and *b* is a chamber sealed with sand *b'* or the like through which the wire is passed, *c*, *c* being guide rollers over which the wire runs 95 on entering the said chamber.

*d* is a rib on the upper part of the chamber *b* for keeping the wire immersed in the sand.

*e* is a tubular chamber through which the 100 wire or the like passes from the chamber *b*; *f*, *f'* are the inlet and outlet respectively in the chamber *e* for the hydrogen gas.

*g* is the galvanizing or tinning chamber arranged in communication with the tubular 105 chamber *e* between the ends thereof, and having a removable top *g'* adapted to be sealed by molten metal of a lower melting point than that forming the bath, and a supply pipe *g''* for the metal forming the bath. 110

*h, h'* are guide rollers for the wire as it enters and leaves the said chamber *g*, and *i, i'* are rollers for guiding the wire beneath the surface of the molten metal in the said 5 chamber, these rollers being carried upon a rod *j* passing through a guide *k* in the top *g'* of the chamber *g* and being adjustable therein in order that the wire passing through the chamber may be immersed to a greater 10 or less extent in the molten metal.

*m* is the chamber from which the wire emerges after the treatment and *o* is the sand level seal therein, this chamber being similar to the chamber *b* and having guide 15 rollers *p, p* over which the wire issues. Where it is desired to merely clean and not to coat the wire *a* as it emerges from the tubular chamber *e*, instead of being conducted

into the chamber *g*, it is fed through the sand seal *q* to the exterior.

20

Claim.

In the scaling and annealing of metals which may be subsequently coated, the process whereby the metal is heated to or above the annealing temperature, in an atmosphere of a reducing gas, present in excess over the amount necessary to reduce the scale or rust to the metallic state, and the said metal at the time of beginning and completing the process is heated to a temperature of from 100° to 150° C.

25

30

SHERARD OSBORN COWPER-COLES.

Witnesses:

H. D. JAMESON,  
J. SHURE.